

Feb. 6, 1962

J. E. CAMP ETAL

3,020,139

ABRASIVE PRODUCT

Filed April 18, 1960

2 Sheets-Sheet 1



FIG. 1



FIG. 3

JOHN E. CAMP  
JOSEF C. MUELLER, JR.  
FREDERICK G. SANDHOLDT  
GEORGE L. HAYWOOD  
INVENTORS

BY *Hugh T. Smith*

ATTORNEY

Feb. 6, 1962

J. E. CAMP ETAL

3,020,139

ABRASIVE PRODUCT

Filed April 18, 1960

2 Sheets-Sheet 2



FIG. 2

JOHN E. CAMP  
JOSEFF C. MUELLER, JR.  
FREDERICK G. SANDHOLDT  
GEORGE L. HAYWOOD  
INVENTORS

BY *Hugh T. Smith*

ATTORNEY

1

3,020,139

## ABRASIVE PRODUCT

John E. Camp, Latham, Josef C. Mueller, Jr., Cohoes, Frederick G. Sandholdt, North Troy, and George L. Haywood, Latham, N.Y., assignors to Norton Company, Troy, N.Y., a corporation of Massachusetts

Filed Apr. 18, 1960, Ser. No. 22,947  
19 Claims. (Cl. 51—295)

The present invention relates in general to polishing or abrading products and in particular to such products utilizing a non-woven textile material as a backing and to methods of making the same.

It has heretofore been proposed to utilize non-woven, felted materials as a media for carrying abrasive grain, the resulting product finding application as a component of a grinding wheel or as a polishing or scrubbing device. Examples of such products are disclosed in U.S. Patent No. 2,335,902 issued to Albert L. Ball, Raymond C. Benner and Romie L. Melton. It has been found, however, that for severe abrading or polishing operations such products find little application although the economics of using a relatively thick (compared to a conventional piece of coated abrasive) backing impregnated with abrasive grain should make such products very desirable for many uses.

Improved products of this general type have been disclosed and claimed in the copending applications of George L. Haywood, Serial No. 782,689, and Serial No. 807,892, filed December 24, 1958, and April 21, 1959, respectively.

Still further improvement has been found possible through the use of a radically different making technique which permits positive retention of the loft of the non-woven backing, accurate control of the amounts of grain and adhesive applied to the backing, improved adhesion between adjacent layers of the backing when convolute bodies thereof are formed, and most importantly, a more uniform dispersal of abrasive grain throughout the non-woven material.

Accordingly, it is an object of the present invention to provide a new method for forming non-woven, abrading or polishing materials.

Another object is to provide an abrasive article of the type referred to above which has more uniform distribution of abrasive throughout.

Additional objects, if not specifically set forth herein, will be readily apparent to one skilled in the art from the following detailed description of the invention.

In the drawings:

FIGURE 1 is a schematic illustration of the method of forming the non-woven, abrasive-containing material of the present invention.

FIGURE 2 is an exploded, idealized view of the abrasive-containing material formed as shown in FIGURE 1, illustrating the disposition of the fibers, the bonding adhesive and the maker adhesive and grain coatings thereon.

FIGURE 3 is a perspective view of one type of abrasive article formed in accordance with the present invention.

Generally, the present invention resides in first treating a non-woven web with a bonding adhesive applied preferably in the form of a spray, resulting in a web capable of being handled without disintegration. Since, as mentioned below, the fibers forming the web are preferably nylon or other synthetic fibers, anti-wetting lubricants are generally present thereon. This resulting anti-wetting property is generally possessed by all such synthetic fibers and, as a result, the adhesive applied by the spray inherently tends to collect at the fiber intersections in the form of globules.

Accordingly, the web first formed consists of many interlaced, randomly dispersed, flexible, tough organic fibers bonded together essentially only at points where they

2

intersect and contact one another by globules of adhesive.

It has heretofore been proposed to form such a web for use as a polishing device by using an abrasive grain-adhesive mixture to form globules at the points of intersection of the fibers. However, to adequately bond abrasive particles to the synthetic fibers and to hold them firmly in place during subsequent abrading operations, the adhesive must be heat-resistant, tough and quite rigid in nature. When used to bond the fibers together, such an adhesive makes the product undesirably harsh and stiff. Likewise, the location of the abrasive particles substantially only at the points of intersection of the fibers is undesirable since the abrading action is much less than is the case of a more uniform distribution of the abrasive along each fiber length. Therefore, in the present case, it is desirable that the "bonding adhesive," as it is hereinafter called, be abrasive-free and that it be elastomeric in nature. The thus-formed web is then subjected to a roll coating operation utilizing an adhesive-abrasive slurry as the coating material. The solvent or dispersant for this second adhesive, which is hereinafter referred to as the "maker" adhesive and which is substantially harder and tougher than the bonding adhesive, is such that it has no or at most only a slight softening effect upon the first-applied bonding adhesive. As a result of these two factors, (1) the use of roll coating and (2) the use of a different solvent or dispersant system for the harder, tougher maker adhesive, an outstanding improvement in the non-woven abrasive product is achieved. The initial loft or three-dimensional characteristic of the web is retained since the bonding adhesive which holds the web in such three-dimensional form is not materially affected by the solvent used in applying the maker adhesive-abrasive coating. Secondly, through the action of roll coating, the maker adhesive tends to deposit along the fibers in the form of elongated strings rather than merely at the points of fiber intersection as is the case with the usual spray application. Some of the maker adhesive surrounds and reinforces the softer, more elastic bonding adhesive at the fiber intersections as well, thus giving a very widespread distribution of abrasive grain throughout the web.

More particularly, and referring now to FIGURE 1 of the drawings, reference numeral 10 designates a web or batt of non-woven material formed from flexible, tough, synthetic organic filaments 11 such as coarse nylon fibres having a diameter of up to about 300 microns. Other synthetic fibres or filaments or mixtures thereof such as "Dacron" (a condensate of dimethyl terephthalate and ethylene glycol), "Orlon" (polyacrylonitrile) or "Dyne" (a copolymer of 40% acrylonitrile and 60% vinyl chloride) may be used as desired and the diameter of the fibres used may also be varied within wide limits, e.g. 25 to 300 microns. As will be seen from the schematic drawing of FIGURE 1, the fibres 11 are formed into desired lengths, e.g. 2 inches or so, by a suitable cutter device generally shown at 12 and deposited upon a moving endless support 13. As the fibres 11 fall to the surface of the support 13, they may be agitated by an air blast from nozzles 14. The fibres 11 tend to fall at various angles to one another and to criss-cross and interlace one with the other in a superposed, random fashion. However, it will be noted that the tendency still is for the length direction of the fibres to lie predominately in the horizontal plane. A web 10 of the desired thickness is built-up—either by regulating the speed of the support 13 and the rate of discharge thereon of the fibres 11 or by the use of additional fibre supplying stations (not shown). The fibres comprising the web 10 are then bonded to one another by a bonding adhesive which may be any of the adhesives discussed in detail below. The bonding adhesive 15 is applied by

spray nozzles 16 which may be stationary or preferably so mounted as to reciprocate back and forth across the web 10. The bonded web 10 then passes through a heating zone 17 to set or cure the adhesive 15. At this point the bonded web has a loft, or three-dimensional characteristic, maintained through the location of the globules of bonding adhesive at primarily the points of intersection of the fibres. It may be and is, in many instances, desirable at this point to reverse the web and again pass it through to spray coat the opposite side of the web with the bonding adhesive.

Experimentation has determined that if the bonding adhesive is substantially softened by subsequent application of additional adhesive, the loft is materially reduced. Accordingly, the next step in the illustrated process, which is the application of abrasive grain to the web is accomplished through the use of a maker adhesive having little or no softening action on the bonding adhesive. Examples of the types of adhesive systems for use in the present method—both maker and bonding adhesives—are given below. Further, it has been determined that much improved adhesive distribution is achieved if the maker adhesive is applied by a roll coater rather than through the use of the conventional spray application. As illustrated, the bonded web 10 is passed through roll coater 18 which consists of a pair of calender rolls 19 and 20, the lower roll 20 rotating in a bath 21 of adhesive-abrasive slurry 22. The maker coat of adhesive and grain thus applied, thoroughly penetrates the web 10 and tends to spread out along the fibers 11 thereof. This is more clearly illustrated in FIGURE 2 of the drawings, hereinafter referred to. The web 10 is then passed through a heating zone 23 to set the maker adhesive. Depending upon the final form in which the web is to be used, the maker adhesive is completely or only partially dried in zone 23. If the material is to be used in flat form, e.g. as discs die-cut from the web, the maker coat is completely dried in zone 23. If, as we prefer, the material is to be formed into convolute discs, the maker adhesive is partially dried so as to remain tacky. As illustrated, the tacky material is then wound into a tight convolute roll 25 as shown at 24 and subjected to further heating in zone 26 to finally cure and dry the maker adhesive. When so treated, the adjacent convolutions are tightly bonded one to the other to essentially form a homogeneous mass. The roll 25 is then cut transversely as shown at 27 to form abrasive articles 28 of the type shown and described below in connection with FIGURE 3 of the drawings.

Referring now to FIGURE 2 of the drawings, an exploded idealized view of the material 10 described in connection with FIGURE 1 is shown. FIGURE 2A shows the general relationship to one another of a group of fibres as laid down to form the web; FIGURE 2B shows the same group of fibres after the spray-applied bonding adhesive has dried thereon; and FIGURE 2C shows the same group of fibres after the roll-coat application of the maker adhesive-abrasive slurry. At the points of intersection 30 of the fibres 31, it will be seen from FIGURE 2B that globules 32 of the bonding adhesive have effectively encased such intersections with a flexible bond. It will be noted that the bonding adhesive 32 tends to settle at the fiber intersections 30 or junctions of the fibers since this adhesive was applied, as described above, by a spray application (usually as a water dispersion). While the bonding adhesive tends to settle substantially at the fiber intersections, occasional globules will adhere along the fibers as indicated at 32'. The maker adhesive 33, on the other hand, is applied by roll coating from a solvent slurry of adhesive and abrasive grain. This adhesive 33 has better wetting properties and the roll coat application tends to coat the maker-adhesive along the fibers as well as at the junctions thereof. Accordingly, as shown in FIGURE 2C the fibers 31 tend to be fairly well coated throughout

their length with the maker adhesive 33 and abrasive grain 34. As illustrated, the maker adhesive-abrasive grain mixture 33—34 tends to form a coating over the globules 32 of the bonding adhesive as well as coating the major portion of each fiber 31.

FIGURE 3 illustrates one form into which the abrasive material of the present invention may be shaped for ultimate use. The article 40 is formed from the roll 25 described in connection with FIGURE 1 by slicing a section normal to the major axis of the roll. As illustrated, the convolutions of material are not visible which is quite common since proper control of tension can vary the roll density to the point where a section such as 40 appears quite homogeneous in nature. The fibers 41 with the abrasive grains 42 held thereto by the maker adhesive 43 provide an excellent abrading or polishing surface. This particular structure is particularly adapted for use as a floor scrubbing pad. Other forms such as rolls or drums for industrial polishing, segments for pot 20 and pan scrubbers, etc., may be formed as desired.

The character of the present product depends upon the two-step adhesive application described above with the second adhesive application being that which bonds the abrasive to the fibers. The second adhesive or "maker" adhesive must, of necessity, be hard, tough and heat-resistant in order to hold the abrasive grain in place on the fibers during the subsequent use of the product in abrading or polishing. The maker adhesive therefore tends to stiffen the fibers. Accordingly, to counteract this tendency, it is essential that the bonding adhesive, which is applied to the fibers before the maker adhesive, be flexible enough to permit flexing and temporary deformation of the product while in use. For example, if the bonding adhesive used is a heat-convertible resin such as a stiff melamine or urea-formaldehyde resin, epoxy-phenolic blend, or the like, a non-resilient, friable product results. Therefore, the bonding adhesive must be relatively flexible and preferably elastomeric in nature. It must also be relatively insoluble in the solvent employed in dissolving the maker adhesive and preferably resistant to alkalis. Accordingly, elastomers must be selected for their relative insolubility in such solvents as methyl isobutylketone, solox, cellosolve acetate and xylene. Preferably, the bonding adhesive is based on a nitrile rubber latex modified to impart solvent resistance. The latices may be modified by the use of curing agents such as zinc oxide, sodium aluminate or by the addition of resins such as phenolics, melamine or urea-formaldehyde. For example, the elastomeric bonding adhesive used in Example 1, below, was a medium butadiene acrylonitrile latex (Hycar 1572 prepared by the B. F. Goodrich Company) having a pH of 8.5 and a particle size of 1000 angstroms. This was blended with a water soluble melamine formaldehyde resin (Resloom HP prepared by Monsanto Chemical Company). Other Hycar latices which may be used include Hycar 1512, 1562 and 1551. Other elastomeric materials such as natural rubber, neoprene or the like may also be used if desired.

The maker adhesives used may vary widely but generally are heat-advancing resinous adhesives based on polyurethanes, phenolics, epoxy resins or the like which adhere well to the synthetic fiber used and which utilize a solvent system to which the bonding adhesive is resistant. Preferably, for use in floor pads or the like, the maker adhesive is also alkali-resistant and is substantially harder and tougher than the bonding adhesive.

Any of the known abrasive grains may be used in making the product of the present invention, e.g. silicon carbide, aluminum oxide, flint, emery, garnet and the like. Generally, the most satisfactory abrasives are silicon carbide, garnet and aluminum oxide. The grain size may likewise be varied within wide limits, with grades 180, 240 and 400 being the most commonly employed sizes for commercial use.

The fibers employed in the present invention are preferably synthetic fibers formed from flexible, tough, alkali-

resistant, organic materials such as the polyamides, acrylates, polyesters, polypropylenes, polyethylene and vinylidene chloride derivatives. The preferred fiber is nylon as discussed above.

The following specific examples of products formed in accordance with the present invention are intended to be illustrative only and therefore only such limitations are intended as may appear in the appended claims.

#### EXAMPLE I

A 40 inch wide web of non-woven coarse nylon fibers—partially drawn producers' waste ranging from 15 to 180 denier and about 1½" in length—was prepared as described above in connection with FIGURE 1, using a conventional Rando-Webber machine and applying a spray coating of an alkali-resistant acrylonitrile-butadiene elastomer in latex form blended with a melamine-formaldehyde resin. The web prior to application of the bonding adhesive weighed 3.6 oz./sq. yd.

##### Bonding adhesive

Parts by weight  
(dry basis)

|                              |     |
|------------------------------|-----|
| Hycar 1572 latex             | 100 |
| Melamine formaldehyde resin  | 15  |
| Stabilizer (Emulphor ON870)  | 1   |
| Amine catalyst AC (Monsanto) | 1½  |

The wet web was then passed through an infra-red oven to make the web tack-free. The reverse side was then sprayed with the same bonding adhesive and given a similar heat treatment. Heating was carried out on each pass for approximately 1 to 3 minutes at 250°-350° F. This effectively drove off the water and cured or partially cured the bonding adhesive to the point where it was relatively solvent-resistant. A total weight of 1.8 oz./sq. yd. of bonding adhesive was applied. Examination of the bonded web indicated that the bulk of the adhesive was deposited in the form of globules at the junctions of the fibers.

The bonded web was then passed at a rate of 10 feet/minute through a padder or roll coater as described above in connection with FIGURE 1 and the maker-adhesive-abrasive slurry applied. In this case the maker adhesive was a polyester-isocyanate prepolymer blend in a solvent system containing methyl isobutylketone, xylene and cellosolve acetate. The abrasive grain (Grit No. 180, silicon carbide) was mixed with this adhesive (Brookfield viscosity of 135 centipoises at 80° F.) in the ratio of about 150% abrasive grain based on the resin solids to form the slurry. The viscosity of the slurry was adjusted to around 950 centipoises at 80° F. at the coating unit with solvent so that good fiber coverage was obtained. Too dense or viscous a slurry would tear or distort the web as it passed through the rolls. About .097 pound of slurry per square foot of material was applied.

##### Maker adhesive—Abrasive slurry

|                                   |                                                                                                      |
|-----------------------------------|------------------------------------------------------------------------------------------------------|
| Mondur CB-60 (Mobay Chemical Co.) | 128.8 pounds (poly-isocyanate formed by reacting toluene diisocyanate with a tri-functional polyol). |
|-----------------------------------|------------------------------------------------------------------------------------------------------|

|                                              |                          |
|----------------------------------------------|--------------------------|
| Fomrez 50 (100% solids) (Witco Chemical Co.) | 38.5 pounds (polyester). |
| Methyl isobutylketone                        | 52.0 pounds.             |
| 180 grit silicon carbide                     | 220.5 pounds.            |

The web was then rolled into jumbo roll form and put into a curing oven. Hot air at 250° F. was blown through the roll for three hours to effect cure of the adhesive. The roll was then ready for processing into such form as might be desired for ultimate use.

#### EXAMPLE 2

In some instances, particularly for fine polishing or buffing operations, the non-woven material formed in ac-

cording with the present invention is utilized without abrasive grain present. Such a product was formed by laying down fifteen denier 1½" staple nylon fibers in the manner described in Example 1 to form a loose non-woven web weighing approximately 2.4 oz./sq. yd. This web was then spray-bonded with an acrylonitrile-butadiene elastomer blended with a melamine-formaldehyde resin as in Example 1. The wet web was heated by passage through an infra-red oven for 1-3 minutes at 300°-350° F. (time dependent upon web speed—usually about 18 feet/minute). The reverse side of the web was then given a similar treatment.

The bonded web was then roll coated with a phenolic resin adhesive (no abrasive) in an alcohol-water solvent system (Brookfield viscosity of 285 centipoises at 80° F.) applied at a web speed of 10 feet/minute and at an amount of about 7¾ pounds resin, on a solids basis, per sandpaper ream (i.e. per 330 square feet). The phenol formaldehyde resin used had a water tolerance of 20 and a gel time at 250° F. at 5.25 seconds. The wet web was then rolled into jumbo roll form and put into a curing oven for 5 hours at 250° F. The finished product was found to be quite satisfactory as a polishing medium for tile floors after being cut into pads of the type illustrated in FIGURE 3.

#### EXAMPLE 3

A web of coarse nylon fibers was made as in Example 1, using as the spray-applied bonding coat a commercial acrylonitrile-butadiene latex binder with no resin modification. The maker adhesive in this case was an epoxy resin (Epon 815 prepared by Shell Chemical Company), and only enough solvent (xylene) was added to the adhesive-abrasive mixture to slightly adjust the viscosity for uniform coating. The adhesive had a Brookfield viscosity of 120 centipoises at 88° F. before the abrasive was added, increasing to 1075 centipoises at 94° F. after the grain was added. The ratio of abrasive to resin and the amounts of slurry coated were as described in Example 1.

The epoxy resin adhesive in the present case was of the low temperature curing type and curing was therefore effected by standing at room temperature after the web had been rolled up into jumbo roll form. This product was then mounted upon suitable bearings and used intact as a wide polishing drum.

From the above description of the present invention, it will be seen that the spray application of a flexible, elastomeric bonding adhesive followed by the roll coat application of a tough, hard, resinous maker adhesive permits the retention of loft and resilience in the resulting non-woven web while at the same time resulting in an improved dispersion of the maker adhesive over the surfaces of the synthetic fibers used in forming the web. Obviously other modifications and variations may be made without departing from the spirit and scope of the invention described therein.

We claim:

1. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a harder, more rigid adhesive applied by roll coating without substantial softening of said elastomeric adhesive.

2. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers sub-

stantially at the points of intersection of said fibers with one another, said adhesive bonding said fibers one to the other so as to form a resilient web; and overlying said elastomeric bonding adhesive and extending further than said bonding adhesive along the length of said fibers, a hard, tough, resinous adhesive applied by roll coating without substantial softening of said elastomeric adhesive.

3. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a harder, more rigid adhesive, said harder, more rigid adhesive being applied by roll coating from a solvent system having relatively little softening effect upon said elastomeric bonding adhesive.

4. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a hard, tough, resinous adhesive, said hard, tough, resinous adhesive being applied by roll coating from a solvent system having relatively little softening effect upon said elastomeric bonding adhesive.

5. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a harder, more rigid adhesive applied by roll coating without substantial softening of said elastomeric adhesive; and a plurality of abrasive grains distributed along said fibers and bonded thereto solely by said harder, more rigid adhesive.

6. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a hard, tough, resinous adhesive applied by roll coating without substantial softening of said elastomeric adhesive; and a plurality of abrasive grains distributed along said fibers and bonded thereto solely by said hard, tough, resinous adhesive.

7. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers

substantially at the points of intersection of said fibers with one another, said adhesive bonding said fibers one to the other so as to form a resilient web; and overlying said elastomeric bonding adhesive and extending further than said bonding adhesive along the length of said fibers, a harder, more rigid adhesive, said harder, more rigid adhesive being applied by roll coating from a solvent system having relatively little softening effect upon said elastomeric bonding adhesive; and a plurality of abrasive grains distributed along said fibers and bonded thereto solely by said harder, more rigid adhesive.

8. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a hard, tough, resinous adhesive, said hard, tough, resinous adhesive being applied by roll coating from a solvent system having relatively little softening effect upon said elastomeric bonding adhesive; and a plurality of abrasive grains distributed along said fibers and bonded thereto solely by said hard, tough, resinous adhesive.

9. An article of manufacture comprising: a three-dimensional open non-woven web having substantial loft and a high proportion of internal voids formed by laying down in superposed random fashion a plurality of relatively short flexible tough synthetic organic fibers; an elastomeric bonding adhesive adhering to said fibers substantially at the points of intersection of said fibers with one another, said adhesive bonding said fibers one to the other so as to form a resilient web; and overlying said elastomeric bonding adhesive and extending further than said bonding adhesive along the length of said fibers, a harder, more rigid adhesive, said harder, more rigid adhesive being applied by roll coating from a solvent system having relatively little softening effect upon said elastomeric bonding adhesive; and a plurality of abrasive grains distributed along said fibers and bonded thereto solely by said harder, more rigid adhesive; said non-woven web being tightly wound upon itself in convolute form while said harder, more rigid adhesive is still tacky to form a self-sustaining cylinder.

10. An article as in claim 9 wherein said cylinder is cut transverse and normal to the long central axis thereof to form a circular pad of non-woven, abrasive-containing material.

11. A method for the manufacture of a non-woven polishing material which comprises: forming a lofty, open, three-dimensional web of flexible, tough, synthetic organic fibers by laying down in superposed random fashion a plurality of relatively short lengths of such fibers; applying to said fibers an elastomeric bonding adhesive, said adhesive tending to concentrate substantially at the points of intersection of said fibers and to bond said fibers one to the other; and applying by roll coating over said elastomeric bonding adhesive without substantially softening the same a harder, tougher adhesive.

12. A method for the manufacture of a non-woven polishing material which comprises: forming a lofty, open, three-dimensional web of flexible, tough, synthetic organic fibers by laying down in superposed random fashion a plurality of relatively short lengths of such fibers; applying to said fibers an elastomeric bonding adhesive, said adhesive tending to concentrate substantially at the points of intersection of said fibers and to bond said fibers one to the other; and applying by roll coating over said elastomeric bonding adhesive without substantially softening the same a harder, tougher adhesive,

said harder, tougher adhesive extending along said fiber lengths as well as overlying said elastomeric bonding adhesive at said points of intersection of said fibers.

13. A method for the manufacture of a non-woven polishing material which comprises: forming a lofty, open, three-dimensional web of flexible, tough, synthetic organic fibers by laying down in superposed random fashion a plurality of relatively short lengths of such fibers; applying to said fibers an elastomeric bonding adhesive, said adhesive tending to concentrate substantially at the points of intersection of said fibers and to bond said fibers one to the other; drying said elastomeric bonding adhesive to a non-tacky state; and thereafter applying by roll coating over said dried elastomeric bonding adhesive without substantially softening the same a harder, tougher adhesive.

14. A method for the manufacture of a non-woven polishing material which comprises: forming a lofty, open, three-dimensional web of flexible, tough, synthetic organic fibers by laying down in superposed random fashion a plurality of relatively short lengths of such fibers; applying to said fibers an elastomeric bonding adhesive, said adhesive tending to concentrate substantially at the points of intersection of said fibers and to bond said fibers one to the other; drying said elastomeric bonding adhesive to a non-tacky state; and thereafter applying by roll coating over said dried elastomeric bonding adhesive without substantially softening the same a harder, tougher adhesive, said harder, tougher adhesive extending along said fiber lengths as well as overlying said elastomeric bonding adhesive at said points of intersection of said fibers.

15. A method for the manufacture of a non-woven polishing material which comprises: forming a lofty, open, three-dimensional web of flexible, tough, synthetic organic fibers by laying down in superposed random fashion a plurality of relatively short lengths of such fibers; applying to said fibers an elastomeric bonding adhesive, said adhesive tending to concentrate substantially at the points of intersection of said fibers and to bond said fibers one to the other; and applying by roll coating over said elastomeric bonding adhesive without substantially softening the same a harder, tougher adhesive containing a plurality of abrasive grains, said harder, tougher adhesive-abrasive grain mixture extending along said fiber lengths as well as overlying said elastomeric bonding adhesive at said points of intersection of said fibers.

16. A method for the manufacture of a non-woven polishing material which comprises: forming a lofty, open, three-dimensional web of flexible, tough, synthetic organic fibers by laying down in superposed random fashion a plurality of relatively short lengths of such fibers; applying to said fibers an elastomeric bonding adhesive, said adhesive tending to concentrate substantially at the points of intersection of said fibers and to bond said fibers one to the other; drying said elastomeric bonding adhesive to a non-tacky state; and thereafter applying by roll coating over said dried elastomeric bonding adhesive without substantially softening the same a harder, tougher adhesive containing a plurality of abrasive grains, said harder, tougher adhesive-abrasive grain mix-

ture extending along said fiber lengths as well as overlying said elastomeric bonding adhesive at said points of intersection of said fibers.

17. A method for the manufacture of a non-woven polishing material which comprises: forming a lofty, open, three-dimensional web of flexible, tough, synthetic organic fibers by laying down in superposed random fashion a plurality of relatively short lengths of such fibers; spraying said fibers of said web with an elastomeric bonding adhesive, said adhesive tending to concentrate substantially at the points of intersection of said fibers whereby said fibers are bonded one to the other and the loft of said web is maintained; drying said elastomeric bonding adhesive to a substantially non-tacky state; and thereafter applying by roll coating a harder, tougher adhesive containing a plurality of abrasive grains to said web without substantial softening of said elastomeric adhesive; said adhesive-abrasive mixture overlying said elastomeric bonding adhesive and extending further than said bonding adhesive along the lengths of said fibers.
18. A method for the manufacture of a non-woven polishing material which comprises: forming a lofty, open, three-dimensional web of flexible, tough, synthetic organic fibers by laying down in superposed random fashion a plurality of relatively short lengths of such fibers; spraying said fibers of said web with an elastomeric bonding adhesive, said adhesive tending to concentrate substantially at the points of intersection of said fibers whereby said fibers are bonded one to the other and the loft of said web is maintained; drying said elastomeric bonding adhesive to a substantially non-tacky state; and thereafter applying by roll coating a harder, tougher, adhesive containing a plurality of abrasive grains to said web without substantial softening of said elastomeric adhesive, said adhesive-abrasive mixture overlying said elastomeric bonding adhesive and extending further than said bonding adhesive along the lengths of said fibers.

19. A method for the manufacture of a non-woven polishing material which comprises: forming a lofty, open, three-dimensional web of flexible, tough, synthetic organic fibers by laying down in superposed random fashion a plurality of relatively short lengths of such fibers; spraying said fibers of said web with an elastomeric bonding adhesive, said adhesive tending to concentrate substantially at the points of intersection of said fibers whereby said fibers are bonded one to the other and the loft of said web is maintained; drying said elastomeric bonding adhesive to a substantially non-tacky state; and thereafter applying to said web by roll coating from a solvent system having relatively little softening effect upon said elastomeric bonding adhesive a harder, tougher adhesive containing a plurality of abrasive grains; said adhesive-abrasive mixture extending along said fiber lengths as well as overlying said elastomeric bonding adhesive.

- 55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8

UNITED STATES PATENT OFFICE

## Certificate

Patent No. 3,020,139

Patented February 6, 1962

John E. Camp, Josef C. Mueller, Jr., Frederick G. Sandholdt, and George L. Haywood

Application having been made jointly by John E. Camp, Josef C. Mueller, Jr., Frederick G. Sandholdt, and George L. Haywood, the inventors in the patent above identified, and The Norton Company, Troy, New York, a corporation of Massachusetts, the assignee, for the issuance of a certificate under the provisions of Title 35, Section 256 of the United States Code, deleting the names of John E. Camp, Frederick G. Sandholdt, and George L. Haywood from the patent as joint inventors, and a showing and proof of facts satisfying the requirements of the said section having been submitted, it is this 4th day of March 1969, certified that the names of John E. Camp, Frederick G. Sandholdt, and George L. Haywood are hereby deleted from the said patent as joint inventors with the said Josef C. Mueller, Jr.

[SEAL]

EDWIN L. REYNOLDS,  
*First Assistant Commissioner of Patents.*